

## UNITED STATES PATENT OFFICE

HANS FRIEDLANDER, OF BERLIN-WILMERSDORF, AND ARTHUR JANSER, OF BERLIN-CHARLOTTENBURG, GERMANY; SAID JANSER ASSIGNOR TO SAID FRIEDLANDER

SUBSTITUTE FOR HARD PAPER, EBONITE, FIBER, AND THE LIKE AND A PROCESS FOR  
MANUFACTURING THE SAME

No Drawing. Application filed June 24, 1925, Serial No. 39,376, and in Austria June 26, 1924.

This invention relates to fibrous materials fully saturated with hard waxes and processes of preparing the same and it comprises as a new material, fibrous materials containing Montan wax hardened by heating to a relatively high temperature or otherwise disseminated therethrough and fully saturating the materials; it further comprises the process in which such fibrous materials are saturated with hardened Montan wax.

In our process, we advantageously impregnate fibrous materials such as cardboard, felt, paper-mâché, etc., with hardened Montan wax, in the molten state, impregnation being continued until the fibrous material is substantially saturated and aided, if desired, by the use of pressure or vacuum.

After cooling, which may take place under pressure, there is obtained an elastic material of sounding hardness, high tensile, compressive and bending strength, with high insulating capacities, which may be easily worked, capable of replacing for many technical purposes the well known technical materials such as ebonite, hard paper and fiber. This is all the more remarkable, as the primary materials, e. g. cardboard and hardened Montan wax, cannot be expected to produce such an effect by themselves, since neither the wax nor the fibrous material possesses one of the qualities specified: cardboard being pliable and of low strength and on the contrary hardened Montan wax being very brittle and exempt of any breaking strength.

This exceptional increase of the properties referred to may be explained by the crypto-cristalline structure of the hardened Montan wax.

It is essential in accordance with the invention that not Montan wax in its original state is used but Montan wax which has been hardened by the addition of small quantities of resins, metallic salts, high-molecular weight acids and the like, or by heating the Montan wax, before or during the impregnation operation, to 200° C. or more. Methods of hardening soft waxes are well known.

The impregnation itself is facilitated and its duration shortened when the fibrous materials treated already contain a part of the hardened Montan wax necessary to completely fill up the pores in a powdered condition or precipitated as a so called wax-sizing.

In this state the materials of course show none of the properties specified according to the idea of the present invention, since the wax particles are dispersed without any coherence between the fibers and are melted together with the molten hardened Montan wax but under the influence of the same during impregnation.

For the impregnation materials of any description and shape made of any fibrous material, such as cardboard, felt, papier-mâché pieces, which, manufactured in any known way, may also contain mineral loading materials, binding materials, &c., are suitable.

A material of specific properties is obtained by the impregnation of materials glued together (lined) to form plates, tubes, &c., in several layers by means of suitable agglutinants such as casein and water glass. Objects manufactured in this way afford an especially high cracking, breaking or bending resistance.

The materials may also undergo, prior to impregnation with hard waxes, a preliminary treatment (preliminary impregnation) with other substances which only partially fill up the pores of the primary material leaving the same partially open for the wax impregnation proper. Hereby the technical properties of the finished materials, e. g. their hardness and strength, in general the mechanical qualities, may be considerably improved.

Compact materials, e. g. highly sized and pressed cardboards are not fit for double impregnation, but for simple wax treatment. A material especially suited for double impregnation is cotton felt as used for filtering.

For the purpose of preliminary impregnation there may be used dissolved or liquid natural or artificial resins, e. g. bakelite or

other substance such as impregnating varnishes, water glass or the like; amongst these stuffs there may be chosen such ones having a hardening effect upon the hard wax used in the second impregnation.

5 The double impregnation affords materials or bodies consisting of three phases or substances or systems completely penetrating each other. This fact may scientifically 10 explain the good mechanical properties of the products obtained.

In consequence of the preliminary impregnation the fibers of the fundamental material are protected against heat in the 15 subsequent impregnation so that with the second impregnation with hardened Montan wax the temperature may be increased.

*Examples*

20 1. Dry cardboard sized with aluminum resinate in a known way is immersed in melted Montan wax at a temperature which is raised from 90 to 230° centigrade and left in the bath until it is completely saturated. Then the plates are allowed to cool with or without pressure applied to.

25 2. Papier-mâché pulp prepared in a known way is mixed with powdered Montan wax and formed into a desired shape. 30 When solidified these articles are treated with melted Montan wax heated to a high temperature as described in the preceding example.

35 3. Cotton felt, e. g. in slabs as used for filters is saturated with a solution of artificial resin in a solvent, e. g. a 40% solution of bakelite, and then dried. The material impregnated in this way is hardened at 140 centigrade in the known way and 40 finally immersed in melted Montan wax heated to a temperature of 230° C. and further treated according to Example 1.

What we claim is:

45 The process of preparing hard sheet material which comprises impregnating felted fibrous material with Montan wax heated to above 200° C.

In testimony whereof we have signed our names to this specification.

50 HANS FRIEDLANDER.  
ARTHUR JANSEN.